

1  
 2,749,226

**DELAY COMPOSITION FOR DELAY ELECTRIC DETONATORS**

Idwal O. Lewis, Ardrossan, Scotland, assignor to Imperial Chemical Industries Limited, a corporation of Great Britain

 No Drawing. Application April 7, 1952,  
 Serial No. 281,029

Claims priority, application Great Britain June 20, 1951

2 Claims. (Cl. 52—2)

This invention relates to improvements in or relating to ventless short period delay electric detonators wherein the delay element consists of a tube containing a delay composition comprising a mixture of red lead and silicon and to delay compositions of the aforesaid kind.

It has previously been proposed, for example in Canadian Patent No. 469,169 to provide a ventless short-period delay electric detonator comprising a shell containing at least one detonating explosive charge, a delay element consisting of a tube containing a fuse composition in contact therewith and an initiating means spaced from said delay element wherein the fuse composition consists of 72-75 per cent by weight of red lead, 30-12 per cent by weight of silicon and 0-18 per cent by weight of an inert diluent, said silicon and inert diluent being in a finely divided form. These compositions are stated to yield delay elements of higher burning speed and greater constancy of burning speed in ventless delay detonators than those consisting of other proportions of red lead and silicon. These fuse compositions, however, suffer from the disadvantage that their burning speeds tend to be too widely scattered about a mean for some purposes, for example for use in a 25 millisecond interval delay series of detonators. Thus using these compositions in delay elements in such a series of detonators, overlapping is liable to occur and this may prevent the attainment of the object of using a number of delay detonators to fire a sufficient number of shots in succession in a suitably restricted time.

The object of the present invention is to provide a delay composition which permits the delay element of a batch of ventless delay electric detonators having a mean delay period of approximately 25 milliseconds to be at least 3 millimetres long and for the deviation of the delay period of each detonator from said mean to be sufficiently small to permit a series of ventless delay detonators having delay intervals of 25 milliseconds to be produced.

It was to be expected that the burning speeds of delay compositions consisting of mixtures of red lead and silicon would generally increase with increase in fineness of the silicon used and also that for any particular degree of fineness of silicon as the silicon content increases from zero the burning speed would increase to a maximum and thereafter diminish and further that the ratio of red lead to silicon which gives maximum burning speed and this maximum burning would differ according to the degree of the fineness of the silicon

used. It was, however, not to be expected that only a narrow range of ratios of red lead to silicon would decrease the deviation of the delay period of the delay element of each delay detonator from a mean delay period to such an extent as to permit a series of ventless delay detonators having delay intervals of 25 milliseconds to be produced. It has now been found by a series of experiments that by selecting the proportions of red lead to silicon so that the red lead is 91-95 per cent by weight and the silicon is 9-5 per cent by weight and by choosing the grain of the silicon so that not less than 90 per cent by weight of said silicon is less than 5 microns and all of it is of size less than 20 microns delay compositions can be produced which are suitable for use in the production of a series of ventless delay detonators having delay intervals of 25 milliseconds.

According to the present invention a ventless short period delay electric detonator is characterised in that the delay composition in its delay element comprises a mixture of 91-95 per cent by weight of red lead and 9-5 per cent by weight of silicon, not less than 90 per cent by weight of said silicon being of particle size less than 5 microns and all of it of size less than 20 microns.

20 A delay composition according to the invention comprises a mixture of 91-95 per cent by weight of red lead and 9-5 per cent by weight of silicon, not less than 90 per cent by weight of said silicon being of particle size less than 5 microns and all of it of size less than 20 microns.

25 By varying the lengths of such delay elements included in the detonators the time intervals between the shots in series or parallel firing may be predetermined.

When these delay compositions are loaded into metal tubes of inner diameter 0.130 inch and outer diameter 0.24 inch in small increments, each increment being pressed at 15 tons per square inch and the so obtained delay elements loaded into electric detonator assemblies the delay elements will have a linear burning speed of approximately 10 milliseconds per millimetre and the variation of delay periods of such assemblies is so small as to permit their use in a 25 millisecond interval delay series of detonators.

30 The degree of fineness of the silicon used may vary widely within the limits prescribed above but is preferably such that at least 95 per cent by weight is of particle size less than 5 microns.

35 In the following table there is recorded the delay times in milliseconds for red lead and silicon compositions according to the invention, i. e. compositions No. 4, and for red lead and silicon compositions not in accordance with the invention, i. e. compositions Nos. 1 to 3 and 5 to 8, when used in delay elements having an inner diameter of 0.130 inch in commercial ventless delay detonators. The table also shows the proportions by weight 40 of the red lead and silicon, the percentage distribution of the particle size in the silicon, and the lengths of the delay elements.

| No. | Composition |         | Length of delay element in mm. | Percentage distribution of particle size in the silicon |             |             |            |          | Delay times in milliseconds |      |      | Scatter, i. e. difference between max. and min. |  |
|-----|-------------|---------|--------------------------------|---------------------------------------------------------|-------------|-------------|------------|----------|-----------------------------|------|------|-------------------------------------------------|--|
|     | Red lead    | Silicon |                                | >35 $\mu$                                               | 20-35 $\mu$ | 10-20 $\mu$ | 5-10 $\mu$ | <5 $\mu$ | Mean                        | Max. | Min. |                                                 |  |
|     |             |         |                                |                                                         |             |             |            |          |                             |      |      |                                                 |  |
| 1   | 70          | 30      | 8.0                            | 3                                                       | 7           | 23          | 31         | 36       | 150                         | 160  | 139  | 21                                              |  |
| 2   | 70          | 30      | 8.0                            | 3                                                       | 7           | 20          | 25         | 45       | 82                          | 123  | 74   | 49                                              |  |
| 3   | 74          | 26      | 8.0                            | 1                                                       | 4           | 20          | 25         | 50       | 83                          | 115  | 68   | 47                                              |  |
| 4   | 93          | 7       | 8.0                            | —                                                       | —           | 2           | 3          | 95       | 72                          | 77   | 67   | 10                                              |  |
| 4   | 93          | 7       | 5.5                            | —                                                       | —           | 2           | 3          | 95       | 50                          | 58   | 45   | 13                                              |  |
| 4   | 93          | 7       | 3.0                            | —                                                       | —           | 2           | 3          | 95       | 25                          | 33   | 15   | 18                                              |  |
| 5   | 93          | 7       | 8.0                            | 4                                                       | 7           | 28          | 23         | 38       | 400                         | 430  | 370  | 60                                              |  |
| 6   | 93          | 7       | 8.0                            | —                                                       | 1           | 4           | 15         | 80       | 105                         | 127  | 90   | 37                                              |  |
| 7   | 70          | 30      | 10.5                           | —                                                       | —           | 2           | 3          | 95       | 65                          | 81   | 52   | 29                                              |  |
| 8   | 80          | 20      | 10.5                           | —                                                       | —           | 2           | 3          | 95       | 50                          | 74   | 45   | 29                                              |  |

The number of observations as a result of which the mean, maximum, and minimum delay times for each delay element was determined was at least 25. It will be appreciated that in a round of shots to be fired at 25 millisecond intervals, the shots will always fire in the correct order when compositions No. 4 are used but may not fire in the correct order when composition No. 2, 3, 5, 6, 7, or 8 is used. Composition No. 1 would be suitable from the point of variability of delay period but to obtain delay periods of 25, 50 and 75 milliseconds, the delay elements would require to be approximately 1.27, 2.54 and 3.81 millimetres long respectively. Such a series of lengths of delay element would, however, not be convenient for use in manufacturing operations.

What I claim is:

1. A delay composition for a delay element, said composition consisting essentially of a mixture of 91% to 95% by weight of red lead and 9% to 5% by weight

of silicon, not less than 90% by weight of said silicon being of particle size less than 5 microns and all of it of size less than 20 microns.

2. A delay composition as claimed in claim 1 where-  
5 in the silicon is of a degree of fineness such that at least 95 per cent by weight is of particle size less than 5 microns.

References Cited in the file of this patent

UNITED STATES PATENTS

|           |             |       |               |
|-----------|-------------|-------|---------------|
| 1,999,820 | Nash        | ----- | Apr. 30, 1935 |
| 2,127,603 | Jones       | ----- | Aug. 23, 1938 |
| 2,586,959 | Kerr et al. | ----- | Feb. 26, 1952 |

FOREIGN PATENTS

|         |        |       |              |
|---------|--------|-------|--------------|
| 469,168 | Canada | ----- | Nov. 7, 1950 |
| 469,169 | Canada | ----- | Nov. 7, 1950 |